

J. BANWELL.

PAVING STRIP.

APPLICATION FILED MAR. 5, 1913.

1,134,939.

Patented Apr. 6, 1915.



Fig. 2



Fig. 3



ATTEST  
E. F. Fisher  
F. C. Musser.

INVENTOR  
By James Banwell  
F. C. Musser, ATTY.

# UNITED STATES PATENT OFFICE.

JAMES BANWELL, OF CLEVELAND, OHIO, ASSIGNOR OF ONE-THIRD TO ROBERT L. BECK,  
OF CLEVELAND, OHIO.

## PAVING-STRIP.

1,134,939.

Specification of Letters Patent.

Patented Apr. 6, 1915.

Application filed March 5, 1913, Serial No. 752,038.

To all whom it may concern:

Be it known that I, JAMES BANWELL, a citizen of the United States, residing at Cleveland, in the county of Cuyahoga and State of Ohio, have invented certain new and useful Improvements in Paving-Strips, of which the following is a specification.

My invention comprises a paving strip having the distinguishing internal and external features substantially as herein shown and described and more particularly pointed out in the claim.

My improved paving strip is designed for use between the paving bricks or blocks of a street and the curb-stone, the object being two-fold; first, to permit expansion and contraction of the paving proper; and second, to maintain a permanent watertight joint and adhesive union between the parts under such expansion and contraction. The strip is also particularly constructed to be water-proof and to sustain high weather temperatures without melting and also to stand an extremely low temperature of weather without materially changing its physical properties, particularly its elasticity and adhesiveness. The strip is also provided with a coating or covering, especially on its wider surfaces, which will permit packing, convenient handling and transporting of such strips and still yield a water-proof and adhesive union of the desired permanency and effect.

In the accompanying drawings, Figure 1 is a perspective view of a section of a pavement and curbing with my improved strip in place therein. Fig. 2 is a perspective view of a single strip comprising my invention. Fig. 3 is a cross section on a larger scale of the paving strip shown in the other views.

As shown, the paving strip consists of a relatively thin and flat piece of elastic and flexible material 2 having beveled end faces 3 which are reversely related. This material is in the main a petroleum residuum, consisting of hydro-carbons, mostly of the paraffin series which have undergone chemical changes through the application of heat and the absorption of oxygen. It is preferably an asphaltic mass of rubber-like texture having a melting point preferably higher than 130° Fahrenheit and embodying certain physical properties to maintain its elasticity and adhesiveness under zero tem-

peratures, even as low as 20° F. below zero. It is also impenetrable to water and not subject to disintegration by water under a temperature less than the melting point given. This material is produced by the distillation of crude oil of certain grades, to eliminate all the volatile portions consisting of gasoline, burning oil and light lubricating oils. The process of distillation is further continued with such modifications as manufacturing requirements dictate, such as diminishing atmospheric pressure in the still, admission of steam and air into the still and into the body of the material contained therein. This asphaltic material is preferably mixed with sand to stiffen the same, and a binder of shoddy-dust or equivalent textile material is also incorporated therewith. Approximately fifty per cent asphaltic material and fifty per cent sand, with about twenty-five per cent shoddy-dust constitutes the mixture and strip, but I do not wish to limit myself to this exact formula.

The strips are molded into any desired length, usually about three to four feet long, and a coating of lime or chalk 4 is applied to one side and sand 5 to the other, or both sides may be coated lightly with lime, or a combined lime and sand covering may be applied. The coating is preferably thin, the primary object being to provide a protective covering to permit the strips to be packed one upon the other for a reasonable length of time without sticking to one another and to allow them to be shipped and handled. The coating being of friable material is loose and removable in a large measure, that is, it may be wiped or knocked off in part prior to laying it in paving operations.

The beveled ends 3 and the top and bottom edges 6 are preferably not coated. However, a thin coating over ends 3 might not prove detrimental to a homogeneous union between the meeting ends of two strips 2 when laid in overlapping relation in the paving, providing a permeable material was used. But by having the ends 3 uncoated and in their natural state, two conducting strips will cohere perfectly and no open joint will be left to permit water and frost to enter and cause trouble.

In laying the strips 2 end to end between the paving and curbing, each alternate strip

- is reversely placed relatively to the adjacent strip to bring the adjacent ends in overlapping relations. This is of further advantage in producing a reasonably quick adhesive union of the strips successively with both the curb and the paving, particularly when one side of the strip is coated with lime and the other with sand, as the asphaltic mass permeates the sand more easily than lime, although it must be also understood that the lime coating is also permeable by the asphaltic mass under the influence of heat to effect a water-tight union with the paving and curbing.
- 15 In paving a street the general practice is to pour and sweep cementitious fluid in the cracks between the bricks or blocks, and this fluid will fill all remaining interstices after an adhesive union by the strip itself with the blocks and curbing has been effected. Sand and lime are materials having the valuable characteristics of uniting with cement and therefore of particular utility in this strip and for the use intended. No 20 water can penetrate through the strip or the sealed joints, and the strip will compress under expansion of the pavement and also stretch when contraction of the paving takes

place without breaking the seal or joints. In brief, my improved paving strip is a 30 marketable product of practical value and utility for the purpose intended, being easily handled and shipped and working economy in paving operations and having all the requisite properties and characteristics to 35 endure heat and cold and sudden changes of weather under long usage to maintain a permanently sealed joint at the curb line regardless of the expansion and contraction of the pavement. 40

What I claim is:

A paving strip adapted to be used between the paving blocks of a street and the curb to allow for expansion and contraction of the pavement and to maintain a sealed 45 joint, and consisting of a solid flat sided body of asphaltic material having beveled ends, the sides of said body being faced with a granular material.

In testimony whereof I affix my signature 50 in presence of two witnesses.

JAMES BANWELL.

Witnesses:

F. C. MUSSUN,  
E. M. FISHER.